

B. TALBOT.  
MANUFACTURE OF STEEL SHAPES.  
APPLICATION FILED NOV. 6, 1912.

1,055,833.

Patented Mar. 11, 1913.

Fig. 1.



Fig. 2.



Fig. 3.



WITNESSES:

Geo. G. Wrenn  
Geo. Wrenn



INVENTOR  
Benz Talbot  
BY  
Charles N. Butler  
ATTORNEY.

# UNITED STATES PATENT OFFICE.

BENJAMIN TALBOT, OF WOODBURN, DARLINGTON, ENGLAND.

## MANUFACTURE OF STEEL SHAPES.

1,055,833.

Specification of Letters Patent. Patented Mar. 11, 1913.

Application filed November 6, 1912. Serial No. 729,766.

*To all whom it may concern:*

Be it known that I, BENJAMIN TALBOT, a British subject, residing at Woodburn, Darlington, Durham county, England, have invented new and useful Improvements in the Manufacture of Steel Shapes, of which the following is a specification.

My invention relates more particularly to the manufacture of railway rails and it has as its primary object to improve the structure of the metal of the usual steel rail so that it shall be free from flaws and defects and possessed of a uniformly tough interior lower in carbon than the outer strata.

Steel rails frequently contain hidden flaws and structural defects, due to blow holes, cavities and segregates, which have resulted in many serious accidents. Usually the carbon in the central part of the upper third of the ingot is higher than in the outer strata, which produces a rail or rails having harder interior sections than the exteriors subject to wear, which is the reverse of the desired conditions. These defects are due to conditions arising in the process of manufacture in which the ingot is formed by pouring the molten steel into a mold and allowing it to solidify without provision compensating for internal shrinkage and the presence of gas confined within the hardened outer strata, and segregation within the upper part of the mass. If usual cold ingots be divided longitudinally, they will be found to contain blow holes or cavities, particularly in the upper third part, either scattered through the mass or, where a powerful deoxidizer has been added to the molten steel, the smaller blow holes are eliminated in great measure and large cavities or pipes are formed in the center of the upper third of the ingot. In the process of cooling, carbon, sulfur and phosphorus segregate and move, as the metal cools, from the outer to the inner parts of the ingots, collecting in excess in the central part of the upper third as a segregate, frequently in seriously objectionable degree. When such ingots are heated to the requisite temperature and rolled, the blow holes and cavities or pipes are found in the finished products as cracks or flaws, since the metal surrounding them cannot be heated to a fluid condition, and the sections in which the excessive segregation has taken place produce sections in the finished products which are de-

fective, more or less of the metal in such sections being brittle and treacherous.

I have found that if an ingot be stripped as soon as practicable after casting, placed in a heating furnace or soaking pit until the solidified envelop has increased in thickness and become sufficiently ductile or plastic to work without cracking or rupturing, and then squeezed while its interior is still in a fluid condition so as to contract its cross sectional area to compensate for shrinkage and eliminate cavities due to confined gas and unequal cooling, it will be found that the interior of the ingot is, due to the condensing lateral pressure, solid in texture, free from blow holes, cavities or pipes except in a limited end portion; that the mass of the central portion of the ingot is lower in carbon than the outer strata; that there is a slight but unobjectionable indication of segregation approximately parallel to and at a short distance from the surface of the ingot; and that there is no segregation within the central mass of the ingot and no objectionable segregation elsewhere.

At the end of the treatment in the soaking pit, the pipe in the upper part of the ingot is partially formed and the metal between the solidified but ductile outer strata and fluid central mass has little coherence, so that when the ingot in this condition is subjected to lateral pressure, as by passing it through a cogging mill, the liquid metal fills the pipe and the contained gases are forced outwardly, passing through or being absorbed by the enveloping metal, while carbon, phosphorus and sulfur diffused through the congealing metal are retained, tests showing these elements in higher degree and distributed in a comparatively uniform manner through the envelop, with a slightly increased amount at a short distance from the surface where a segregate, if substantial in character, would be least objectionable. An ingot of this character, when rolled or drawn, will produce rails, beams and other shapes or products having comparatively pure and tough interiors combined with comparatively hard exteriors, without the usual defects and with substantial economy of material, since there is required to be removed but a small crop or discard as practically the whole ingot is solid.

In carrying out my invention, I prefer to treat the molten steel, either before or af-

ter it is poured into the ingot mold, with metallic aluminum, or other deoxidizer, such as silicon, ferro-silicon, silico-manganese or ferro-titanium, for the purpose, primarily, of effecting initially the elimination of small blow holes disseminated throughout the envelop of the upper portion of the ingot and to hasten the stiffening of the metal.

As the objectionable cavities and segregation take place in the upper third of the ingot, I may confine the squeezing operation for the purpose of eliminating the cavities and disseminating the segregates to such upper third or only the upper part of the ingot.

In steel which has been treated by an electrical refining process, the amount of segregation observed is usually very small, but the cavities form in the same way as in steel made by the Bessemer or Siemens processes, and it is my purpose to produce ingots and the products thereof without the defects resulting from such cavities.

While it is not essential to do so in all cases, the ingots will generally, after having been subjected to the squeezing operation, be returned to the heating furnace or soaking pit, to effect a more nearly equal and desirable temperature and condition throughout the mass of the metal prior to rolling or finally forming the desired shape.

In the accompanying drawings, Figure 1 is a longitudinal sectional view of a steel ingot after stripping when it has a comparatively thin envelop of solid metal surrounding a fluid body; Fig. 2 is a longitudinal sectional view of the same after it has been heated in a soaking pit for such time and at such temperature that the envelop has become sufficiently thick and sufficiently soft to work without rupturing; Fig. 3 is a longitudinal sectional view representing an ingot or bloom that has resulted from squeezing the ingot shown in Fig. 2 by the application of lateral pressure thereto so as to reduce its cross-sectional area; Fig. 4 is a transverse sectional view of a rail produced by rolling the ingot or bloom shown in Fig. 3; Fig. 5 is a transverse sectional view of an I-beam rolled from an ingot or bloom like that shown in Fig. 3; and Fig. 6 is a longitudinal sectional view representing an ingot having the cross section of only its upper part reduced to eliminate cavities and force the segregates outwardly.

The ingot A, shown in Fig. 1, is say 20" wide at the bottom and has an envelop *a* which may be 1" thick, such envelop being too thin and hard for satisfactory contraction by rolling or squeezing to reduce the cross section of the ingot while its central part *a'* is still fluid.

The ingot B, shown in Fig. 2, results from heating the ingot A until there is produced the comparatively soft or ductile and

thick envelop *b* containing the fluid central mass *b'*, at the top of which the cavity *b''* will have formed, the envelop being, say, 3" thick.

The ingot or bloom C, shown in Fig. 3, is the product resulting from giving the ingot B several passes in a cogging mill or otherwise squeezing it so as to reduce its cross sectional area, eliminate the cavities or confine them to a restricted part of the top, and provide the comparatively pure central part *c* surrounded by the strata *c'* of somewhat higher carbon, together with phosphorus and sulfur (if any), there being generally a noticeable but unobjectionable stratum of segregation along the inner part *c''* of the strata *c'*. That is to say, as shown by averaging sections of a typical ingot, where the central part *c* contained an average of .50% carbon, .02% phosphorus and .03% sulfur, an outer stratum *c'* near the edge of the ingot contained an average of .70% carbon, .03% phosphorus and .04% sulfur, and a stratum *c''* between the foregoing parts an average of .80% carbon, .04% phosphorus and .06% sulfur.

It will be understood that there is no distinct or abrupt line of demarcation between the strata, which term is used here with reference to zones containing different amounts of the elements, the change in the amounts of the elements through the several strata being gradual.

The rail D, shown in Fig. 4, is the product produced by rolling the ingot or bloom C, the rail having the comparatively pure and soft central part *d* and the harder exterior *d'* providing a tough body combined with a hard wearing surface.

The I-beam E, shown in Fig. 5, is likewise provided with the comparatively pure and soft central or body part *e* with a slightly harder surface *e'*.

The ingot F, shown in Fig. 6, has its upper part only reduced in cross section, with resulting elimination of cavities and diffusion of the matter which would otherwise form a segregate in the center of such upper part. The lower part of the ingot will be found to be in the usual condition, the center *f* of the upper part will be found comparatively pure, and the outer strata *f'* will be found to have the segregates diffused therethrough, particularly through the parts thereof adjacent to the central part *f*.

It will be understood that while I have given specific illustrations of dimensions and conditions, in order to explain my invention by example, such illustrations are merely by way of example and not limiting features of my invention.

Having described my invention, I claim:

1. The process which comprises subjecting a steel ingot having a fluid center to a heating operation at such temperature and

for such time as to so soften and increase the thickness of the envelop that it can be worked without rupturing; then subjecting said ingot to lateral pressure so as to reduce 5 its cross-sectional area, eliminate cavities, and diffuse the segregates; and finally rolling said ingot into a rail.

2. The process which comprises subjecting an ingot composed of steel that has been 10 treated with a deoxidizer to a heating operation while its center is still fluid, at such temperature and for such time as to soften the envelop and increase its thickness so that it can be worked without rupturing; 15 then subjecting the ingot to lateral pressure so as to eliminate cavities therein and diffuse carbon from the center thereof through the strata exterior to the fluid center; and finally drawing said ingot into a 20 shape having a refined central part lower in carbon than the outer part.

3. The process which comprises subjecting an ingot composed of steel that has been 25 treated with a deoxidizer to a heating operation while its center is still fluid, at such

temperature and for such time as to soften the envelop and increase its thickness so that it can be worked without rupturing, subjecting the ingot to lateral pressure so as to eliminate cavities therein, and finally rolling 30 the ingot into a rail.

4. The process which comprises subjecting an ingot composed of steel to a heating operation while its center is still fluid, at such temperature and for such time as to 35 soften the envelop and increase its thickness so that it can be worked without rupturing; then subjecting such ingot to lateral pressure so as to eliminate cavities therein; reheating said ingot for such time and at 40 such temperature as may be required to fit it for rolling into a shape, and finally rolling said ingot into a shape.

In witness whereof I have hereunto set my name this 4th day of November, 1912, 45 in the presence of the subscribing witnesses.

BENJAMIN TALBOT.

Witnesses:

Jos. G. DENNY, Jr.,  
GEO. A. CRENNEY.